

June 11, 1940.

G. R. LONG

2,203,915

ICE TRAY

Original Filed Feb. 26, 1937



Fig. 1



Fig. 2



Fig. 3

INVENTOR.

GEORGE R. LONG.

BY

Spencer, Hardman and Zeh.  
HIS ATTORNEYS.

## UNITED STATES PATENT OFFICE

2,203,915

## ICE TRAY

George R. Long, Dayton, Ohio, assignor to General Motors Corporation, Dayton, Ohio, a corporation of Delaware

Application February 26, 1937, Serial No. 127,927  
Renewed November 7, 1939

## 4 Claims. (Cl. 62—108.5)

This invention relates to refrigerators and particularly to freezing devices employed in mechanically refrigerated household refrigerator cabinets.

5 In order to obtain fast freezing of a substance to be frozen in the evaporator of a household refrigerator cabinet it has been customary to employ an ice tray and grid structure therefor both of which are constructed of or formed from 10 metal. Because of inherent characteristics of water to adhere to metal surfaces the separation of ice blocks from such trays and grids has presented many problems. The metal of such trays and grids are ordinarily somewhat porous 15 or pitted throughout the surfaces thereof with which water contacts during freezing and such surfaces tend to cause the water to spread over and adhere to the metal. The water upon being frozen in contact with these metal surfaces sticks 20 or bonds to the metal. My invention is directed to the provision of surfaces of metal ice trays and grid structures therefor, with which water contacts, that will be substantially repellent to the water to thereby eliminate spreading of its 25 molecules upon contacting a tray and grid walls to thus prevent bonding the ice thereto.

An object of my invention is to provide an improved ice tray and grid structure therefor so as to facilitate the removal of ice blocks therefrom.

30 Another object of my invention is to coat the walls of a metal tray and grid structure therefor with a waxy substance to thereby render the walls water repellent to prevent bonding of ice thereto.

35 In carrying out the foregoing objects it is a still further and more specific object of my invention to provide a substantially permanent wax coat on the walls of a metal tray and grid structure therefor which coat consists of a mixture of carnauba wax and a micro-crystalline mineral wax having a melting point of the order of 175° F.

40 Further objects and advantages of the present invention will be apparent from the following description, reference being had to the accompanying drawing, wherein a preferred form of the present invention are clearly shown.

In the drawing:

45 Fig. 1 is a top plan view of an ice tray and a grid structure positioned in the tray having my invention embodied therein;

50 Fig. 2 is a longitudinal vertical sectional view of the tray and grid disclosed in Fig. 1 and taken on the line 2—2 thereof; and

55 Fig. 3 is an enlarged sectional view of one of

the webs of the grid structure illustrating a coating applied thereover in accordance with the invention.

Referring to the drawing, for illustrating my invention, I have shown in Figs. 1 and 2 a metal ice tray 10 having upstanding and outwardly converging walls 11 defining a relatively shallow pan-like member adapted to receive a removable metal grid structure or mold member 12. The metal tray 10 and grid or mold 12, employed to 10 divide the interior of the tray into a plurality of ice block compartments, may be of any desired form or construction but are preferably constructed in accordance with the tray and grid structure disclosed in the copending application 15 of Donald H. Reeves, Serial No. 98,213 filed Aug. 27, 1936. The grid structure in the present disclosure therefore comprises a plurality of transverse walls 14 that are movable relative to a longitudinal wall 15 by movement of a lever 16 20 pivotally attached to the grid to break the ice blocks or cubes 17, frozen in the tray and grid, first from the tray 10 and thence from the grid structure 12, after separating the grid together with ice adhering thereto from the tray as fully described in the copending application referred to. It is the primary purpose of my invention to improve the construction and facilitate the operation of removing ice blocks or cubes from a tray grid structure particularly of the type 25 disclosed in the foregoing identified copending Reeves application.

The tray 10 and walls 14 and 15 of grid 12 of the present disclosure are formed from or constructed of sheet aluminum since this material is of light weight, strong and a good conductor of heat. It has been found that this material will, in the course of extended use, oxidize, corrode and become tarnished or discolored and therefore the wall surfaces of the grid are treated 30 to eliminate as far as possible such discoloring due to oxidation and corrosion. The tray 10 and grid or mold 12 are therefore treated in a manner which causes the formation of an aluminum oxide and/or hydrate coat on the exposed 35 wall surfaces thereof and which coat resists discoloring and tarnishing and is pleasing in appearance. The method of coating the wall surfaces of the tray and grid is known to those skilled in the art as an anodical treatment or 40 anodizing process and is at present being widely carried out commercially, therefore no further detailed description of this method is believed necessary herein. It is well known that this 45 anodical or anodizing treatment of ice trays and 50

5

10

15

20

25

30

35

40

45

50

55

grids provides a surface on the aluminum which is relatively porous, pitted and rough. Thus by treating the aluminum trays and grids in the manner described these trays and grids are provided with wall surfaces that can be readily impregnated or coated with a suitable substance that will destroy or eliminate the porosity or roughness of the surfaces and render these wall surfaces water repellent.

10 Others have, prior to my invention, endeavored to improve and facilitate removal of ice blocks from metal tray or grid walls by plating and highly polishing these walls. It is true that the plating and high polish of tray and grid walls has destroyed their porosity and roughness but these walls have not necessarily been rendered water repellent by the plating thereof and consequently water or ice will bond thereto. Thus plating and polishing of the tray and grid walls 15 does not materially facilitate the operation of removing ice blocks therefrom.

My invention is specifically directed to the provision of a wax coating on metal ice tray and grid walls, and particularly tray and grid walls 20 anodized as hereinbefore described, that will be substantially permanent in water repellent characteristics to thereby facilitate removal of ice therefrom. A coating of carnauba wax, which is amorphous and melts at a temperature between 175° and 195° F., applied to the walls of ice trays and grids has been found to render the walls water repellent and this coating is relatively permanent during extended operations of removing ice therefrom. However, since this wax 25 is of a vegetable origin, difficult to obtain and, in addition imported into this country, its use in a pure or undiluted state is too costly for application to trays or grids on a productive basis. Since the use of carnauba wax alone for coating 30 trays and grids is prohibitive it is desired to employ another wax, possessing characteristics somewhat similar to the characteristics of carnauba wax, to dilute and mix with the carnauba wax for reducing the cost of the coating material to thereby render the application of a wax mixture containing carnauba to ice trays or grids 35 practical as to quantity production.

I have discovered that a wax which is a by-product of crude oil, obtained from the mass of waxes that are left in the oil after distilling off gasoline and kerosene therefrom, and which is micro-crystalline in form and of a considerably higher melting point as compared to paraffin is suitable for mixing with carnauba wax for my 40 purpose. This mineral wax is plentiful, of low cost and is clearly distinguishable from paraffin by having a finer crystalline structure and having a melting point of approximately 50° higher than paraffin. In actual tests this mineral wax has been found to melt at a temperature of from 170° to 180° F. as compared to the melting point of from 120° to 130° F. for most grades of paraffin. Ordinarily this mineral wax is mixed with carnauba wax in the production of automobile, 45 furniture and floor polishing waxes and is employed therein to dilute and soften same so that the polishing wax can be readily "worked" and more easily applied to surfaces to be polished. This mineral wax also contains water repellent 50 characteristics similar to carnauba wax and therefore provides a suitable substance to be mixed with carnauba wax to reduce the cost of providing an effective water repellent coating on articles. I have found that in addition to reducing the cost of the coating material the mix-

ing of this mineral wax with carnauba wax provides a more permanent wax coat and is therefore better for the purpose of accomplishing the objects of my invention than a coating consisting of carnauba wax alone.

My invention therefore resides in the provision of a coating on metal surfaces of ice trays and grids which comprises a mixture of a micro-crystalline mineral wax and carnauba wax. This wax mixture applied to the metal walls of an 10 ice tray or grid forms a smooth coating there-over and facilitates removal of ice blocks therefrom due to the water repellent characteristics thereof. It is known that a mixture of carnauba wax and paraffin will produce a water repellent 15 coating for ice trays and grid structures but it is believed that the larger crystalline characteristics of paraffin in this mixture prevents the mixture from adhering permanently to the metal because such a coating is quickly "broken down" 20 and is therefore removed little by little from metal tray or grid walls to thus become ineffective for its intended purpose. However, by employing a micro-crystalline mineral wax of the type herein disclosed for mixing with carnauba 25 wax the entire mixture is of a substantially amorphous nature and is not as readily broken down or removed from the tray and grid walls. A coating consisting of 50% carnauba wax and 50% of the micro-crystalline mineral wax has 30 been found to remain on metal ice tray and grid walls indefinitely and throughout many operations of removing ice blocks from the tray and grid. While this 50-50 mixture coating has been 35 found to be highly satisfactory it is to be understood that mixtures consisting of from 50% to 75% of the mineral wax and from 50% to 25% of carnauba wax will provide a substantially permanent water repellent coating for the metal walls of trays and grid structures and will greatly 40 facilitate the removal of ice therefrom. Obviously the melting point of the mixtures will vary in accordance with the percentage of the two waxes employed therein.

I have illustrated in Fig. 3 of the drawing the 45 metal grid or mold wall 14 having an aluminum oxide or hydrate coat formed or provided there-on by anodizing the grid as previously explained. A wax coating, illustrated at 19, is shown as being applied over the aluminum oxide or hydrate 50 coat on the grid structure 12. While I have illustrated a portion of the grid 12 having my invention applied thereto it is to be understood that the entire grid structure and the tray is to be provided with the wax coating 19. This wax 55 coating 19 preferably consists of 25% carnauba wax and 75% of the micro-crystalline mineral wax which has a melting point of the order of 175° F. It is to be understood that I do not wish to be limited to the specific proportions of the 60 two wax constituents of the wax coat 19 referred to for the reason that other proportions of the wax have been found to be satisfactory. The substantially amorphous wax coating 19 is relatively permanent and is water repellent therefore water will not adhere thereto during freezing thereof and the ice will not become bonded to the grid walls. Obviously therefore the operation of moving certain of the grid walls relative to certain other walls thereof, during the act 65 of removing ice blocks from the grid structure, in the manner fully disclosed in the copending Reeves application hereinbefore referred to, is greatly facilitated. By eliminating bonding of ice blocks to the grid walls less force is necessary 70

to actuate the ice removing lever and deformation of these walls is prevented to thereby permit the walls to be constructed of relatively thin sheet aluminum.

5 I will now describe one method of applying the wax coat 19 to the tray 10 or to grid 12 in order to carry out my invention. The substantially amorphous wax, consisting of any desired proportion of the micro-crystalline mineral wax 10 and carnauba wax, is melted in a suitable container at a temperature dependent upon the proportions of the wax in the mixture. The tray and grid, which have previously been anodized, to be coated with the wax is submerged in the 15 molten wax and permitted to remain therein for approximately ten minutes to insure that all parts thereof are thoroughly coated. The molten wax penetrates into the pores or crevices of the aluminum oxide or hydrate coat on the tray or 20 grid while being submerged in the wax bath to thereby impregnate the tray and grid with a wax coat. The tray or grid is then removed from the molten wax bath and cooled. Ordinarily there is a sufficient amount of excess wax 25 on the tray or grid to necessitate removal thereof. Therefore the tray or grid is placed in an oven and reheated to a suitable temperature to cause the wax to flow to thereby remove any excess wax therefrom while the desired amount 30 clings or adheres to the tray or grid walls in the form of a thin film thereover. This thin film of wax is both in and on the anodized coating on the tray or grid. If desired the tray or grid may be rotated or whirled to throw off excess wax during reheating of the wax. The tray or grid may, if desired, be heated by hot air forced thereover under pressure to remove excess wax therefrom. While I have described one 35 method of applying the wax coat to a tray or grid structure it is to be understood that other methods may be adopted in carrying out the objects of my invention.

It will be apparent from the foregoing that I have provided an improved ice tray or grid or both in that I have rendered the water contacting surfaces thereof repellent to water to thereby prevent bonding of ice thereto. My improved tray and grid greatly facilitates the operation of removing ice blocks therefrom and permits the 40 structures to be constructed of relatively thin metal because the force necessary to cause separation of ice from the tray or grid is minimized. I wish it to be clearly understood that by describing the mineral wax in the present disclosure as a micro-crystalline or substantially amorphous wax having a melting point of the 45 order of 175° F. I thereby distinguish this wax from paraffin which is also a mineral wax but which has a more distinct and definite crystalline form and a substantially lower melting point.

60 While the form of embodiment of the invention

as herein disclosed, constitutes a preferred form, it is to be understood that other forms might be adopted, all coming within the scope of the claims which follow.

What is claimed is as follows:

1. A freezing device for refrigerating systems comprising a metallic tray adapted to contain a substance to be congealed or frozen and having a substantially permanent water repellent wax coating over at least the surfaces thereof to be 10 contacted by the substance, said coating including a mixture of carnauba wax and a substantially micro-crystalline mineral wax having a melting point of the order of 175° F. as distinguished from paraffin and capable of repeated cleansing 15 in liquid at a temperature of from 140° to 170° F.

2. A freezing device for refrigerating systems comprising a metallic tray adapted to contain a substance to be congealed or frozen and a metallic grid structure disposed therein and dividing the interior thereof into a plurality of compartments, said tray and said grid structure each having a substantially permanent water repellent wax coating over at least the surfaces thereof to be contacted by the substance to be congealed or 20 frozen, said coating including a mixture of carnauba wax and a substantially micro-crystalline mineral wax having a melting point of the order of 175° F. as distinguished from paraffin and capable of repeated cleansing in liquid at a temperature of from 140° to 170° F. 25

3. A freezing device for refrigerating systems comprising a metallic grid structure for disposition in a tray adapted to contain a substance to be congealed or frozen to thereby divide the interior of the tray into a plurality of compartments, said grid structure having a substantially permanent water repellent wax coating over at least the surfaces thereof to be contacted by the substance to be congealed or frozen, said coating including a mixture of carnauba wax and a substantially micro-crystalline mineral wax having a melting point of the order of 175° F. as distinguished from paraffin and capable of repeated cleansing in liquid at a temperature of from 140° 30 to 170° F. 35

4. A freezing device for refrigerating systems comprising a metallic tray member adapted to contain a substance to be congealed or frozen and a metallic grid member disposed in the tray 40 and dividing the interior thereof into a plurality of compartments, one of said members having a water repellent coating over the metal surfaces thereof to be contacted by the substance, said coating consisting of a mixture of from 50% to 55% carnauba wax and from 50% to 75% of a substantially micro-crystalline mineral wax as distinguished from paraffin and having approximately a 50° higher melting point than paraffin. 45

60 GEORGE R. LONG.